

Dec. 17, 1940.

C. SPAETH

2,225,239

FILAMENT

Original Filed Aug. 14, 1936



*Fig. 2.*



*Fig. 4.*



*Fig. 5.*



Inventor

Charles Spaeth

Kenway & Witter

Attorney

## UNITED STATES PATENT OFFICE

2,225,239

## FILAMENT

Charles Spaeth, Flushing, N. Y.

Original application August 14, 1936, Serial No. 96,040. Divided and this application April 18, 1939, Serial No. 268,571

11 Claims. (Cl. 176—40)

This invention consists in a non-sag filament of tungsten wire for use in incandescent or other electric lamps. This application is a division of my application Ser. No. 96,040 now Patent No. 5 2,165,310, granted July 11, 1939, in which the process of making the new filament is disclosed and claimed.

Tungsten wire filaments as heretofore constructed, especially of the coiled coil type, have 10 required special treatment to prevent sagging due to crystalline displacement when operated at the temperature of incandescence in electric lamps. The treatment formerly necessary has required heating of the filament wire at a temperature 15 between 1600 and 1700° C. in order to settle the tungsten crystals permanently in shape. Such treatment has been difficult because furnaces capable of operating at such high temperatures have a short life and are not readily available as 20 commercial equipment.

Other expedients relied upon in producing non-sag tungsten filaments have required the use of additives such as thorium oxide, rare earth metal oxides, rare earth metal nitrides which are 25 expensive to procure or require considerable skill and experience in working.

I have discovered that a satisfactory non-sag filament may be produced from substantially pure tungsten wire or commercial tungsten wire 30 by certain steps of procedure which obviate the difficulties above discussed. In accordance with the process of my invention the structure of the tungsten wire is reinforced by forming a ferrous, nickel or other reinforcing alloy in the wire. This 35 may be readily effected by a series of steps well adapted for processes of commercial manufacture and at little expense and may be advantageously combined with a heat treatment of the filament wherein a preliminary and partial 40 settling of the crystalline structure of the tungsten is effected at a temperature of about 1000° to about 1300° C., followed by a final heating at higher temperature after the filament has been mounted permanently in the lamp in which it is 45 to serve.

I have found it possible to produce a tungsten wire filament having a satisfactory crystalline adjustment of the tungsten wire by subjecting the filament for an interval of from 1 to 10 50 minutes to a temperature of about 1000° to about 1300° C. which is a temperature easily secured in commercial furnaces. The treated filament is then cooled and its mandrels removed and it is mounted in its position in an incandescent lamp, 55 surrounded by the usual argon or nitrogen gases,

heated to a temperature below the temperature used in the previous firing in the furnace and then rapidly raised to a temperature, for example, of approximately 2700° C. for a 100 to 500 watt filament. At about this temperature the 5 final or complete settling of the crystalline structure takes place whereas for filaments of smaller capacity a somewhat lower temperature will suffice.

Preferably the preliminary heating is carried 10 out in an atmosphere of nitrogen, hydrogen or other non-oxidizing gas and in the presence of iron, nickel or some other element having a lower melting point and a higher vapor pressure than tungsten. Under such circumstances a small 15 amount of the iron or other metal is vaporized and deposited upon surface portions of the filament. The low melting point metal may be present as a core upon which the tungsten wire is wound with suitable mandrel and pitch ratios in 20 order to produce sufficient preliminary strains in the tungsten wires and mandrel wires during the coiling operations in coiling single, or coiled coils or triple coils and upon which is deposited simultaneously with the preliminary step of the heat 25 treatment, an iron or other metal film. Iron may also be made available being electrolytical deposition or may be plated upon the surface of the tungsten wire by any satisfactory plating process. As a practical matter it is convenient to deposit 30 a slight excess amount of iron or nickel upon the surface of the tungsten wire, and the surplus may be subsequently removed by a suitable acid solvent. If an iron or nickel core has been employed, this may be dissolved at the same time 35 and only so much iron is left in the filament as has entered into the molecular interstices of the tungsten structure.

The filament is completed by subjecting it to 40 steps which complete the settling of the tungsten crystals and cause the iron or nickel or other metal to be interalloyed with the tungsten. These two changes of physical characteristics may be effected by mounting the filament in the lamp in which it is to be finally used, then raising 45 the filament to a temperature slightly below that at which the previous heating step left off, and finally rapidly raising the temperature of the filament to approximately 2700° C. This may be conveniently effected by placing the filament 50 in electric circuit, first at a potential of about 20 volts, and then raising the potential rapidly to approximately 120 volts, under which condition the filament is raised to incandescent and goes through the changes above discussed, however, 55

it is also possible to apply the 120 volts to the lamp immediately if desired.

The filament of my invention is applicable with special advantage for use as a triple coil filament of the general character disclosed in my co-pending application Ser. No. 15,605, filed April 10, 1935. The fact that the process of making the filament of my invention, in settling or stabilizing the structure of coiled coil filaments, requires lower temperature in the heat treatment of the metal compared to other previously known processes of making coiled coil filaments using molybdenum wire mandrels, makes the filament wire less brittle than heretofore. 10 The addition of the reinforcing alloy of iron or the like reduces the rate of evaporation of the tungsten and this in turn reduces the tendency of blackening the bulb by vaporized deposit from the filament and therefore results in a better 15 lumen maintenance than it has been possible to secure from lamps heretofore known.

These and other features of the invention will be best understood and appreciated from the following description of a preferred embodiment 25 thereof and of one manner in which the process may be carried out, as illustrated in the accompanying drawing, in which—

Fig. 1 is a sectional view, somewhat diagrammatical in form, of a furnace with a number of 30 filament blanks in process of treatment therein,

Fig. 2 is a diagram suggestive of the electrical heating step of the process,

Fig. 3 is a view in perspective showing a 35 mounted coiled filament,

Fig. 4 is a view in elevation on a greatly enlarged scale of a portion of a triple coiled filament, and

Fig. 5 is a sectional view on a still larger scale showing a filament coiled upon its mandrel and 40 coated with an iron deposit shown in a somewhat exaggerated diagrammatical form.

The filament with suitable mandrel ratios and pitch ratios in order to produce sufficient preliminary strains in the tungsten wires and mandrel 45 wires during the coiling process is first coiled in the shape in which it is to be eventually used in the finished lamp, for example coiled coils or triple coils. If a filament of the single coil type is required, tungsten wire 41 may be coiled 50 about an iron mandrel 40 as suggested in Fig. 5. In preparing a double or for example a triple coiled filament the tungsten wire 31 may be first coiled or twisted about a tungsten mandrel wire 30 to form the primary coil, as shown in Fig. 4. 55 The primary coil may then be coiled about an iron mandrel to form secondary coils 32 and the secondary coils, with the enclosed mandrels, may be coiled about another iron mandrel to form tertiary coils 33. A coil of this character is 60 illustrated in Fig. 4.

Having shaped the filament as above outlined, a number of the filament blanks 18, after the conventional cleaning process, are placed in tray 13 and inserted in a high temperature furnace, 65 such for example as that illustrated in Fig. 1. This furnace is one of a type which is commercially available and comprises an outer casing 10 in which is placed a muffle 11 of alundum or other porous and highly refractory material. A 70 heating coil 12 for the muffle is conventionally represented in Fig. 1. The casing 10 is provided with an inlet pipe 14 at the upper left hand corner and with an outlet pipe 15 at its lower right hand corner by means of which non-oxidizing gases, such as nitrogen or hydrogen, or 75

mixtures may be supplied to the furnace so that the heat treatment of the filament blanks may be carried out in a non-oxidizing, inert atmosphere. It will be understood that the material of the muffle 11 is sufficiently porous to permit 5 the gas to permeate it. The filament blanks 18 in single, double or triple coiled form are laid side by side in a tray 13 of molybdenum or material which is not affected by the temperature of the furnace.

Having placed the filament blanks 18 in the furnace as above explained the temperature of the furnace is raised to a temperature between about 1000° and about 1300° C. and the filament blanks subjected to this temperature for a period of about 1 to 10 minutes in an atmosphere of nitrogen or hydrogen preferably which has been passed through a water bath so that it has picked up some moisture. As already explained this step of the process may be carried out in a 10 commercial furnace readily available and having a long life under the circumstances of use outlined.

It will be noted that during this step of the treatment the tungsten wire is wound upon a 25 core of iron, nickel or the like, of a lower melting point and a higher vapor pressure than the tungsten. Accordingly, at a firing temperature of about 1000° to about 1300° C. a small amount of core material is vaporized and deposited upon 30 the surface of the tungsten wire. It is sufficient to state here that during this step of the treatment the amount of vaporized core material represents a very small part of the total mass of the tungsten wire or filament.

The heat treated blanks are now removed 35 from the furnace and allowed to cool. They are then immersed in a suitable acid, for example hydrochloric for iron, and the iron core or cores or other metal cores dissolved. At the same 40 time any excess amount of iron or other metal which may have been deposited upon the wire of the coil is also removed and the film reduced to a thin ferrous film or other metal films intimately associated with the surface structure of 45 the tungsten.

Having now subjected the filament blanks to a preliminary heat treatment which is effective 50 partially to settle the crystalline structure of the tungsten, the filaments are given the final shape under which they are to operate and mounted as suggested in Fig. 3. In this figure the coil filament 20 is shown as supported by hooks above the end of a glass rod 21 which projects from the press 23 of the lamp. Lead wires 22 are sealed into the press 23 and connected to the ends of the filament. The filament with its mount is sealed into a lamp bulb, not shown, in the usual manner, the bulb is exhausted and filled with argon gas, an argon-nitrogen mixture or the like and then connected in electric circuit. The filament is now electrically heated to a temperature somewhat below that at which the preliminary heat treatment left off, i. e. approximately to 1200° C. If the filament is intended for an 120 volt lamp the initial voltage of the circuit may be 20 volts as suggested in Fig. 2, and in any case an initial voltage is used which will produce the desired heating condition, however, if desired the full 120 volts can be 60 applied to the lamp immediately.

Having brought the filament to an initial temperature of approximately 1200° C. the voltage is raised gradually and progressively to a point at which the filament is heated to approximately 75

2700° C. at which temperature a complete settling of the crystalline structure takes place and also a complete alloying of the iron or nickel or other metal film with the tungsten of the filament. This final heat treatment of the coil may be effected in a period of about one second to about one minute as suggested in Fig. 2.

Fig. 5 is suggestive of the alternative step of electrolytically providing the coiled filament with a coating of iron, nickel or the like. In this instance the tungsten wire 41 coiled upon a mandrel 40 is immersed in a solution of ferrous chloride and sodium tungstate and placed in an electric circuit as the cathode of a plating system. The iron from the solution is thus deposited in a film or coating 42 upon the core 40 and the coil 41. Subsequently the thickness of the coating may be reduced to a surface film, or merely to traces of iron in the surface structure of the tungsten, and it is this iron which is subsequently alloyed with the tungsten by the heat treating steps above set forth.

It may be noted that if an ordinary coiled coil filament is heated to about 1000° to 1300° C. and the mandrels on which it was wound are dissolved by an acid, the coil does not maintain its shape but is likely to alter in pitch, turns per inch, internal diameter, etc., because the temperature to which it has been subjected is too low to settle the crystalline structure of the wire.

In order to accomplish settling of ordinary coiled coils with molybdenum mandrels, temperatures of 1500° C. to 1800° are required, hence the use of molybdenum wire mandrels instead of iron mandrels. The result is that under these circumstances the coil will uncoil itself partially and acquire a distorted shape. The process of my invention as above described is fully effective in settling the crystalline structure of the tungsten so that the coils will maintain their form as originally determined by the coiling machine and all this is effected without requiring a furnace treatment of over 1300° C.

Among the numerous advantages of the filament of my invention is that it is more ductile and less brittle than filaments of this kind heretofore known. When the crystalline structure of a tungsten filament is stabilized at a temperature of 1600° to 1700° C. it is rendered brittle to an extent that causes an objectionable amount of breakage due to vibration in handling, in mounting, or in shipment. The preliminary heat treatment at lower temperature, followed by the final treatment at higher temperature in accordance with my novel process results in a more ductile product well adapted to withstand the shocks and vibrations of handling and shipping.

Another important advantage is in increased life of the filament. This is due to the fact that the metal alloyed with the surface of the tungsten wire substantially reduces the rate of vaporization of the filament material in use. This not only reduces waste from the filament itself but reduces blackening of the bulb and thus increases the useful life of the lamp to a marked extent as well as its burn-out life compared on a basis of equal initial efficiency in lumens per watt with lamps heretofore known.

I have described my invention having in mind particularly filaments for 100 to 500 watt lamps and while the temperatures and time intervals mentioned are satisfactory for the treatment of such filaments, it will be understood that some variation in these respects is permitted and ex-

pected. For example, in treating filaments for smaller lamps a final temperature of 2000° to 2400° C. may be adequate in the finished lamp. The time of treatment moreover may vary from a few seconds to several minutes depending somewhat upon the size of the filament being treated.

While it is desirable in general to carry out the heat treatment of the filament in a non-oxidizing atmosphere, it may be advantageous in some cases to include a small amount of water vapor, particularly for the purpose of removing any graphite lubricant which may be present upon the surface of the tungsten wire. If water vapor is present it is decomposed into hydrogen and oxygen and the oxygen will immediately combine with any traces of graphite present on the wire forming carbon monoxide or carbon dioxide which are washed out of the furnace by the hydrogen. This not only cleans the wire but prevents the formation of surface carbides which tend to make the filament brittle.

Having thus described my invention, what I claim as new and desire to secure by Letters Patent is:

1. A filament for an electric lamp comprising a tungsten wire coiled in helical form and permeated by an interalloy of iron produced by first coiling the tungsten wire upon an iron core, then heating to cause some iron from the core to become deposited upon the coil, then dissolving the core, and finally heating to cause the remaining iron and tungsten to become alloyed.

2. A filament comprising a tungsten wire coiled in helical form and permeated by an interalloy of iron imparting non-sagging characteristics to the helix and produced by heating the coiled helix on an iron core simultaneously to effect a partial settling of the crystalline structure and to cause the deposition of iron upon the surface of the wire, cooling the filament, removing the iron core, and then heating it sufficiently to effect a further settling of its crystalline structure and to cause the iron thereon to become alloyed with the tungsten.

3. A coiled ductile filament for a 110 volt to 120 volt lamp, comprising tungsten wire coiled into a helix and permeated by an interalloy of iron and produced by coating the coiled helix with iron, heating it to a temperature between 1000° C. and 1300° C. allowing it to cool, removing the excess iron, and then electrically heating it by including it in a circuit wherein the potential is raised from approximately 20 volts to approximately 120 volts.

4. A filament comprising tungsten wire coiled into a helix and permeated by an interalloy of the iron-nickel group and produced by depositing a surface film of a metal of the iron-nickel group upon the coiled helix, heating the coated helix to a temperature between about 1000° C. and 1300° C., cooling the helix, removing the deposited metal, then again heating it to approximately 1200° C., and finally raising said temperature to above 2000° C., thus imparting a non-sagging character to the filament.

5. A filament comprising a tungsten wire coiled into a helix and permeated by an interalloy of ferrous metal, the filament having been produced by winding the tungsten wire on a core of ferrous metal having a lower melting point and a higher vapor pressure than tungsten, firing the coil to cause some of the core metal to vaporize and be deposited upon the coiled tungsten wire, then cooling the coil, dissolving the ferrous metal

core, and finally heating to a temperature alloying the two metals together.

6. A non-sagging filament comprising tungsten wire coiled in the form of a helix and permeated by an interalloy of ferrous metal, and produced by coating the coil with ferrous metal of a lower melting point and higher vapor pressure than tungsten, heating the coated helix to a temperature of about 1000° to about 1300° C., allowing the helix to cool and then alloying said metal and tungsten by including the helix in an electric circuit wherein the potential is sufficient to heat the wire thereof to about 2000° to 2700° C.

7. A coiled coil filament for electric lamps comprising a tungsten wire coiled in the form of primary and secondary helices and permeated with an interalloy of iron, and produced by winding the wire upon a tungsten core in a primary helix, winding the primary helix with its core upon an iron core, heating to cause some iron from the iron core to become deposited upon the tungsten wire of the filament, removing the iron core, and then further heating to cause the remaining iron to become alloyed with the tungsten wire.

8. A ductile non-sagging filament comprising a tungsten wire coiled in the form of primary and secondary helices and permeated with an interalloy of iron, and produced by winding the tungsten wire upon a refractory core to form a primary helix, winding the primary helix with its core upon an iron core to form a secondary helix, winding the secondary core upon another iron core to form a tertiary helix, heating to cause iron from said core to be deposited upon the tungsten wire of the filament, removing the iron cores, and then further heating to cause the remaining iron to become alloyed with the tungsten wire.

9. A non-sagging filament comprising a tungsten wire coiled in the form of primary and secondary helices and permeated by an interalloy of iron, and produced by winding the tungsten wire upon an iron core to form a primary helix, 5 winding said helix with its core upon a second iron core, heating to cause some iron from the iron cores to be deposited upon the tungsten wire helices thus formed, removing both the iron cores, and then further heating to cause the remaining 10 iron to become alloyed with the tungsten wire of the helices.

10. A ductile non-sagging filament comprising a tungsten wire coiled in the form of primary and secondary helices and permeated by an interalloy 15 of a ferrous metal and produced by winding the tungsten wire upon a ferrous metal core to form a primary helix, winding said helix with its core upon a second ferrous metal core, heating to cause metal from the cores to be deposited upon 20 the tungsten wire helices thus formed, removing both metal cores, and then further heating to cause the remaining metal to become alloyed with the tungsten wire.

11. A coiled coil filament for an electric lamp 25 comprising a tungsten wire coiled in the form of primary and secondary helices and permeated by an interalloy of metals of the nickel-iron group, produced by coiling the tungsten wire upon metal cores of the nickel-iron group, then heating to 30 cause some metal from the cores to become deposited upon the wire to effect simultaneously a partial settling of the crystalline structure of the tungsten wire, removing the metal cores, and then heating it sufficiently to effect a further setting 35 of its crystalline structure.

CHARLES SPAETH.